

# United States Patent

[19]

[11] 3,919,581

Datta

[45] Nov. 11, 1975

[54] THORIA-YTTRIA EMISSION MIXTURE  
FOR DISCHARGE LAMPS

3,485,343 12/1969 Jorgensen ..... 313/218 X  
3,530,327 9/1970 Zollweg et al. ..... 313/346 R

[75] Inventor: Ranajit K. Datta, East Cleveland,  
Ohio

## FOREIGN PATENTS OR APPLICATIONS

252,476 2/1970 U.S.S.R. ..... 313/218

[73] Assignee: General Electric Company,  
Schenectady, N.Y.

Primary Examiner—Saxfield Chatmon, Jr.

[22] Filed: July 12, 1974

Attorney, Agent, or Firm—Ernest W. Legree;  
Lawrence R. Kempton; Frank L. Neuhauser

[21] Appl. No.: 488,109

[52] U.S. CL. ..... 313/345; 313/346; 313/311;  
313/218

## ABSTRACT

[51] Int. CL<sup>2</sup> ..... H01J 1/14; H01J 19/06

An improved emission material particularly useful as a coating on the metallic electrodes of metal halide lamps consists of a solid solution of yttrium oxide in the thorium oxide lattice. Enhanced maintenance including less shifting of color rendition with life is achieved. Preferred proportions are 5 to 20 mole percent of  $Y_2O_3$  in  $ThO_2$  prefired into a single-phase solid solution.

[58] Field of Search ..... 313/345, 346, 311, 218

## References Cited

### UNITED STATES PATENTS

2,460,739 2/1949 Francis ..... 313/346 R  
3,364,375 1/1968 McCarty ..... 313/346 R  
3,372,297 3/1968 Pearsall et al. ..... 313/345 X

7 Claims, 4 Drawing Figures



Fig. 1



Fig. 2



Fig. 3



Fig. 4



# THORIA-YTTRIA EMISSION MIXTURE FOR DISCHARGE LAMPS

## BACKGROUND OF THE INVENTION

High intensity discharge lamps, such as high pressure mercury and metal halide vapor lamps have established themselves as valuable lighting sources. Although one can expect relatively high efficacy as measured in lumens per watt from these lamps, starting and maintenance have remained a problem and a high voltage is generally required to start the electrical discharge.

Considerable effort has been expended in attempts to lower the voltage required to establish the arc. The thermionically emitting tungsten electrodes used in most discharge lamps have a coating of an emission material in the form of a refractory powder mixture to lower the work function in order to start the arc at lower voltage. The process of lowering the starting voltages by applying lower work-function materials on the electrode surface is known as "activation" and an extensive literature exists on cathode activation theory and practice. Concerning cathodes of interest for discharge lamps, the literature includes the following references: E. S. Rittner, Philips Res. Reports, 8, 184 (1953); J. M. Lafferty, J. Appl. Phys., 22, 229 (1951); D. M. Speros, J. Electrochem. Soc., 106, 791 (1959).

The search for better electrode activation materials has been a continuing one. Rare earth oxides including  $\text{ThO}_2$  and  $\text{Y}_2\text{O}_3$  have been used separately or together as emission mix in high intensity discharge lamps on account of their low work function, low vapor pressure and chemical compatibility with the lamp components and arc materials. Some metal halide lamps containing  $\text{NaI}$ ,  $\text{TlI}$  and  $\text{InI}$  as arc materials used a mechanical mixture of  $\text{ThO}_2$  and  $\text{Y}_2\text{O}_3$  with four rare earth oxides for the activation material. Such emission mix containing six oxides mechanically mixed was unsatisfactory, in fact less satisfactory than  $\text{ThO}_2$  alone. According to U.S. Pat. No. 3,530,327 — Zollweg et al., rare earth oxides are most useful in high intensity discharge lamps in which the halides of the same rare earths are used as arc materials, that is, as the materials through whose vapors the arc discharge takes place. In all of these previously known cases, a rare earth oxide or a mechanical mixture of one or more of these oxides (including  $\text{ThO}_2$  and  $\text{Y}_2\text{O}_3$ ) was used as emission mix.

## SUMMARY OF THE INVENTION

The object of my invention is to provide a new emission material having improved characteristics and in particular better maintenance than what has been available up to now.

In accordance with my invention I provide a solid solution of yttrium oxide  $\text{Y}_2\text{O}_3$  in the thorium oxide  $\text{ThO}_2$  lattice, such material forming an improved electron emission material having enhanced maintenance and constancy of color rendition when used for electrode activation in metal halide lamps. The amount of  $\text{Y}_2\text{O}_3$  can range from a small amount effective to improve emission characteristics up to about 50 mole percent. I have found the range from 5 to 20 mole percent of  $\text{Y}_2\text{O}_3$  dissolved in  $\text{ThO}_2$  to be optimum.

## DESCRIPTION OF DRAWINGS

FIG. 1 is a side view of a metal halide lamp in which the arc tube electrodes are activated with emission mix according to the invention.

FIG. 2 is a graph comparing the maintenance of lamps embodying the invention with that of conventional lamps using thorium oxide for electrode activation.

FIG. 3 is a graph comparing the maintenance of lamps embodying the invention with that of lamps using a mechanical mixture of six oxides.

FIG. 4 is a section of a CIE chromaticity diagram comparing the life color line of the lamp of the invention with that of a conventional thorium oxide activated lamp.

## DETAILED DESCRIPTION

The emission material of the present invention is a solid solution of  $\text{Y}_2\text{O}_3$  in the  $\text{ThO}_2$  lattice which may be prepared as follows:

Weigh appropriate amounts of  $\text{Y}_2\text{O}_3$  and  $\text{Th}(\text{NO}_3)_4 \cdot 4\text{H}_2\text{O}$  and dissolve the mixture in dilute nitric acid.  $\text{Th}(\text{NO}_3)_4 \cdot 4\text{H}_2\text{O}$  is soluble in water at room temperature, whereas  $\text{Y}_2\text{O}_3$  dissolves in warm dilute nitric acid. These two materials may be dissolved separately and the solutions mixed together later. The mixed solution should be chilled in a refrigerator for several hours. The metal ions (Th, Y) now can be precipitated as oxalates by slowly adding a supersaturated solution of oxalic acid to the chilled nitrate solution kept in an ice bath. The nitrate solution should be constantly stirred to keep oxalates from forming lumps. The precipitate is now filtered, thoroughly washed and dried at 120°C for several hours. The fine precipitate contained in a platinum crucible is ignited to oxides at 900°C for several hours. The cooled oxide mixture is now ground, blended and reheated at 1500°C for 3-4 hours.

The material resulting from the foregoing preparation shows only one phase, namely  $\text{ThO}_2$  solid solution, under X-ray diffraction analysis. It is well known that the solubility of  $\text{Y}_2\text{O}_3$  in the  $\text{ThO}_2$  lattice increases with the final sintering temperature (V. Subbarao et al., J. Amer. Ceramic Soc., Vol. 48, No. 9, 1965). Thus at 1500° and 1600°C, about 12 and 20 mole percent of  $\text{Y}_2\text{O}_3$ , respectively can be dissolved in the  $\text{ThO}_2$  lattice.

The maintenance of the  $\text{ThO}_2$  emission mix begins to improve as soon as the minutest amount of  $\text{Y}_2\text{O}_3$  is incorporated into the lattice. Thus the amount of  $\text{Y}_2\text{O}_3$  can range from a small amount effective to improve emission characteristics up to about 50 mole percent which is the largest amount which can be incorporated into  $\text{ThO}_2$  in practice. Depending upon the fineness of grinding, the thoroughness of mixing and the reaction time and temperature, less than all of the  $\text{Y}_2\text{O}_3$  may go into solid solution in the  $\text{ThO}_2$ . In such case, the resultant material is a mixture of  $\text{Y}_2\text{O}_3$  and solid solution of  $\text{Y}_2\text{O}_3$  in  $\text{ThO}_2$ . It is the latter material that has the improved characteristics. I have found the range from 5 to 20 mole percent of  $\text{Y}_2\text{O}_3$  dissolved in  $\text{ThO}_2$  as a single phase solid solution to be optimum.

To activate an electrode, the sintered material is mixed with acetone, alcohol or some other organic binder into a slurry and milled for several hours to form a homogeneous suspension of appropriate particle size. The metallic electrode is coated with the emission material by dipping it into the suspension up to a predetermined level; it is then allowed to dry and any loose emission material is brushed off. The amount of the emission material on the electrode surface varies according to the sizes of the lamp (wattage), arc cham-

ber, cathode etc., and can be adjusted by controlling such factors as the density of the suspension and the particle size. The organic binder is burned off and the electrode degassed by thoroughly baking and sintering in the temperature range from 1200° to 1900°C in a vacuum environment prior to incorporation into the arc tube.

FIG. 1 shows an otherwise conventional metal halide lamp 1 of 400 watt size in which my improved emission material may be used. It comprises an outer glass envelope 2 containing a quartz arc tube 3 having electrodes 4, 5 sealed into opposite ends. The arc tube contains an ionizable filling comprising mercury, sodium iodide, thallium iodide, indium iodide and an inert starting gas such as argon. As illustrated, the electrodes may consist of two layers of tungsten wire turns wound over tungsten shanks 6, 7 which are connected through the usual molybdenum foils to inleads 8, 9. The electrodes are coated with the ThO<sub>2</sub> - Y<sub>2</sub>O<sub>3</sub> emission mix which also desirably fills the interstices between turns in the two layers. The arc tube inleads are connected to outer leads 10, 11 sealed through press 12 of stem 13 of outer envelope 2. The outer leads in turn are connected externally to the contact surfaces of screw base 14 attached to the neck end of the envelope.

Metal halide lamps using my emission material show better maintenance and higher efficiency than prior art lamps. In FIG. 2, solid line 20 represents the maintenance of 400 watt lamps such as illustrated in FIG. 1 using the ThO<sub>2</sub> - Y<sub>2</sub>O<sub>3</sub> emission material of the invention while broken line 21 represents that of control lamps using pure ThO<sub>2</sub> as emission mix. Many other high intensity discharge lamps are described in the literature and the ThO<sub>2</sub> - Y<sub>2</sub>O<sub>3</sub> material of the present invention can be used as a long-life source of thermionic electrons in these lamps.

In FIG. 3, solid line 22 shows the maintenance of 400 watt lamps such as illustrated in FIG. 1 using the emission mix of the invention, compared with that of lamps made with the previously mentioned mechanical mixture of six oxides represented by broken line 23.

In addition to enhanced maintenance, the emission material of the invention also shows improved color and less shifting of color rendition from lamps using it. In FIG. 4 which is a section of the 1931 Commission Internationale d'Eclairage chromaticity diagram, solid

line curve 24 represents the color rendition with life of a lamp embodying the invention using the ThO<sub>2</sub> - Y<sub>2</sub>O<sub>3</sub> emission mix, while broken line curve 25 represents that of a conventional lamp using pure ThO<sub>2</sub>. The parenthetical numbers next to the turning points give the lamp life in hours at those points. It will be seen that the lamp according to the invention has less shift in color from 100 to 4000 hours, and less reversal in color from 4000 to 8000 hours. The change in the lamp according to the invention also tends to parallel the black body locus which is a desirable characteristic.

What I claim as new and desire to secure by Letters Patent of the United States is:

1. An electrode for an arc discharge device comprising a refractory metal substrate and an electron emissive material carried thereon comprising a solid solution of Y<sub>2</sub>O<sub>3</sub> in ThO<sub>2</sub> wherein the proportion of Y<sub>2</sub>O<sub>3</sub> is in the range from a small amount effective to improve emission characteristics up to about 50 mole percent in ThO<sub>2</sub>.

2. An electrode as in claim 1 wherein the proportion of Y<sub>2</sub>O<sub>3</sub> is in the range from 5 to 20 mole percent in ThO<sub>2</sub>.

3. A high pressure electric discharge lamp comprising a light-transmitting envelope having refractory metal electrodes sealed into opposite ends and containing an ionizable medium including mercury, metal halide and an inert gas at low pressure, and an electron emissive material carried on said electrodes comprising a solid solution of Y<sub>2</sub>O<sub>3</sub> in ThO<sub>2</sub> wherein the proportion of Y<sub>2</sub>O<sub>3</sub> is in the range from a small amount effective to improve emission characteristics up to about 50 mole percent in ThO<sub>2</sub>.

4. A lamp as in claim 3 wherein the proportion of Y<sub>2</sub>O<sub>3</sub> is in the range from 5 to 20 mole percent in ThO<sub>2</sub>.

5. A lamp as in claim 3 wherein the refractory metal electrodes comprise turns of tungsten wire wound around a tungsten shank and the electron emissive material is coated on said turns and lodged in the interstices between turns.

6. A lamp as in claim 5 wherein the proportion of Y<sub>2</sub>O<sub>3</sub> is in the range from 5 to 20 mole percent in ThO<sub>2</sub>.

7. A lamp as in claim 6 wherein the ionizable filling includes sodium, thallium and indium iodides.